

## UNITED STATES PATENT OFFICE

ARTHUR R. GRAHAM, OF SEAGIRT, NEW JERSEY, ASSIGNOR TO HANSON-VAN WINKLE-MUNNING COMPANY, OF MATAWAN, NEW JERSEY, A CORPORATION OF NEW JERSEY

## ZINC ALUMINUM ANODE FOR ELECTRODEPOSITION OF ZINC

No Drawing. Application filed February 20, 1931. Serial No. 517,307.

This invention relates to anodes for use in the electrodeposition of zinc in both acid and cyanide baths.

Modern practice in the electrodeposition of metals from solution recognizes important advantages in supplying the metal and maintaining the composition of the electrolyte by the employment of soluble anodes of the metal to be deposited. The use of soluble anodes is usually more economical than introducing the metal in the form of soluble salts of the metal, and furthermore tends to maintain the metal content and acidity of the bath more uniform.

In the electrodeposition of zinc from acid baths, for example, the use of pure zinc anodes, which are soluble in the bath, has led to certain difficulties due partly to the fact that such an anode is chemically soluble in the bath even when no external voltage is applied, with the result that a serious loss of metal occurs during idle periods, and even during the electroplating operation the corrosion or solution of the anode occurs at a greater rate than the deposition of the metal upon the cathode. Consequently, the metal content of the bath increases and the acidity of the bath diminishes. The indicated anode efficiency of pure zinc anodes may in a given case be in the neighborhood of 107%, and suspended particles of metal or sludge freed from the anode find their way to the cathode where they adhere as inclusions to the detriment of the electrodeposit both with respect to its appearance and with respect to its protective quality on the article being plated. The indicated cathode efficiency due to such inclusions is also frequently found to be higher than 100%.

Many of the disadvantages of pure zinc anodes in acid baths are also present to some extent in the use of such anodes in cyanide baths.

My invention has for its object to provide an improved soluble anode for use in the electrodeposition of zinc, from either acid or cyanide baths.

In accordance with my invention the anode comprises zinc with a small addition of aluminum. The zinc and aluminum are prefer-

ably fused together as an alloy or intimate homogeneous mixture, and then cast in molds or otherwise formed. The proportion of aluminum to zinc may vary from, for example, 25% to about 5% of aluminum, but I usually employ between 25% and 1% aluminum.

The addition of small quantities of aluminum to zinc confers upon the anode important chemical and electrochemical properties. It reduces the rate of chemical solution of the anode, reduces the indicated anode efficiency, reduces the formation of sludge, improves the grain structure of the anode, causes the anode to corrode more evenly, brings about an approximate equalization of anode and cathode efficiencies without the occurrence of objectionable inclusions of sludge and suspended matter in the electrodeposit, and maintains the metal content and acidity of the solution much more uniform than in the use of pure zinc anodes. The electrodeposit, when using zinc anodes containing aluminum, is of better appearance and texture and offers better protective properties on the electroplated article.

Comparative tests of anodes composed of zinc with additions of aluminum, and anodes composed of substantially pure zinc, showed in the case of acid baths, for example, an anode efficiency of 106.9% with the addition of .27% aluminum to the zinc, an anode efficiency of 104.7% with an addition of .37% aluminum to the zinc, and an anode efficiency of 101.5% with an addition of .74% aluminum to the zinc, whereas four samples of pure zinc showed anode efficiencies ranging from 106% to 107.6%. An addition of .27% aluminum to pure zinc lowered the cathode efficiency from 101.7% (average of three values) to 101%. As compared with a pure zinc anode, an anode of zinc containing .74% aluminum showed noticeably less gassing while hanging idle in the solution than an anode of pure zinc. The metal content of the solution showed after forty-eight hours run a large increase when using pure zinc anodes, and a very slight decrease with small additions of aluminum to the zinc anode. In the same time the acidity of the bath showed substantial decrease when using pure zinc

- anodes and negligible decrease, or even a slight increase, when using anodes of zinc with small additions of aluminum. The grain structure on corrosion showed much finer in the case of the zinc anodes containing small additions of aluminum than in anodes of pure zinc. The sludge formation was also greatly reduced in the case of anodes containing small additions of aluminum.
- 5 10 Each test was conducted with the anode and cathode areas equal.

From the above observations it will be seen that the various factors are subject to control by varying the proportion of aluminum to zinc in the anode, and that the most desirable conditions are obtained with the addition of from .25%, say, to .75% aluminum to pure zinc.

I claim:—

- 20 1. A zinc anode having a small content of aluminum amounting to less than 5%.
2. A zinc anode containing from .25% to 1% aluminum.
3. A zinc anode containing from .25%  
25 to .75% aluminum.

ARTHUR K. GRAHAM.

30

35

40

45

50

55

60

65